

1

3,556,840

**METHOD FOR IMPROVING THE FLAME RETARDANT PROPERTIES OF A CELLULOSIC MATERIAL**  
 Giuliana C. Tesoro, Dobbs Ferry, N.Y., assignor to J. P. Stevens & Co., Inc., New York, N.Y., a corporation of Delaware

No Drawing. Continuation-in-part of application Ser. No. 672,412, Sept. 15, 1967, which is a continuation-in-part of application Ser. No. 620,109, Mar. 2, 1967. This application Mar. 15, 1968, Ser. No. 713,317

Int. Cl. C09k 3/28; C09d 5/18

U.S. Cl. 117—137

8 Claims

**ABSTRACT OF THE DISCLOSURE**

Cellulosic textile materials are rendered flame-retardant by treating the textile material with an N-(oxymethyl)-3-(dialkylphosphono)propionamide, e.g., N-(hydroxymethyl)-3-(diethylphosphono)propionamide, and an acid catalyst and heating to insolubilize the amide compound, and thereafter treating the material with a poly(oxymethyl) melamine, e.g., tris(hydroxymethyl)melamine, and a peroxide such as hydrogen peroxide and heating to insolubilize the melamine compound. The resulting product, which desirably contains 0.5 to 1.8 weight percent phosphorus, based upon the cellulose, and sufficient nitrogen to render the cellulose flame-retardant, retains the soft hand, strength and air permeability characteristic of the untreated textile.

This application is a continuation-in-part of copending application Ser. No. 672,412 filed Sept. 15, 1967, which in turn was a continuation-in-part of application Ser. No. 620,109 filed Mar. 2, 1967, now abandoned.

This invention relates to flame-retardant cellulosic textiles and to methods for their production. More particularly this invention relates to cellulosic fabrics which have been rendered flame-retardant with little adverse effect on the physical properties of the fabric.

It has long been known that flame-retardant properties may be imparted to cellulose, particularly in a textile form, by treatment with phosphoric acid or compounds capable of forming phosphoric acid or its anhydride on burning. However, these methods are generally unacceptable due to series degradation of the cellulose as well as lack of durability of the treatment.

More recently treatments employing organophosphorus compounds have been developed in an effort to provide flame retardance without concurrent damage to the cellulose and to render the phosphorus-containing agent resistant to removal during laundering. Although many of these treatments are in commercial use today, none has been completely successful due to the high cost of the organophosphorus compound and the high degree of add-on of organophosphorus compound required to provide flame-retardant properties.

Still more recently, it has been discovered that organic nitrogen is a synergist for phosphorus-induced flame retardance in cellulose, and thus allows the use of reduced amounts of organophosphorus compound. For example, when 6- to 10-ounce cotton fabric is treated with an organophosphorus compound little or no flame-retardant effect is observed until at least about 1.5 weight percent phosphorus, based on cellulose, is present, and acceptable flame-retardant properties are not achieved until the phosphorus content is at least about 2 percent. By incorporating sufficient organic nitrogen into the treatment, however, excellent flame-retardant properties can be obtained at phosphorus contents as low as about 0.2 weight percent, despite the fact that organic nitrogen compounds alone are not flame-retardant agents. In such treatments the

2

amount of nitrogen which is required increases as the phosphorus content decreases.

Because very few phosphorus-containing compounds also contain nitrogen in amounts sufficient to aid flame retardancy at low total add-on, it has been found necessary to employ organo-nitrogen compounds having high nitrogen contents, such as the poly(oxymethyl)melamines, in combination with the phosphorus-containing compound. One problem with the use of such organonitrogen compounds has been their tendency to cross-link the cellulose and thereby adversely affect properties such as hand, strength and the like. It has been discovered in accordance with the present invention that a desirable degree of flame retardance can be obtained without adverse effect on cellulose properties when an N-(oxymethyl)phosphonopropionamide is employed as the phosphorus-containing compound and the amide and the melamine compounds are applied to the cellulose in a specific sequence.

Briefly, the method of the present invention comprises treating cellulose with an N-(oxymethyl)phosphonopropionamide in an amount sufficient to provide the desired phosphorus content, insolubilizing the amide by acid-catalyzed reaction with the cellulose, and thereafter treating the cellulose with a poly(oxymethyl)melamine in an amount sufficient to provide the desired degree of flame retardance and insolubilizing the melamine compound, preferably a poly(hydroxymethyl)melamine, by wet fixation employing a peroxide.

By the term "oxymethyl," as employed in the present application, is meant hydroxymethyl or lower alkoxy-methyl. By the terms "lower alkyl" and "lower alkoxy," are meant linear or branched chain alkyl and alkoxy groups containing up to about 6 carbons, and preferably up to about 2 carbons, such as methyl, ethyl, isopropyl, tert-butyl, methoxy, ethoxy, isopropoxy, tert-butoxy and the like. By the term "lower alkenyl" is meant alkenyl groups of up to 6 carbons, preferably allyl. By the term "halogen" is meant a halogen having an atomic number of 17 to 53, inclusive, with chlorine being preferred.

N-(oxymethyl)phosphonopropionamides which are employed in accordance with the present invention are represented by the formula:



wherein R is lower alkyl or halogen-substituted lower alkyl; R<sup>1</sup> is hydrogen or lower alkyl; and R<sup>2</sup> is hydrogen, lower alkyl or lower alkenyl; R is preferably alkyl and R<sup>1</sup> and R<sup>2</sup> are preferably hydrogen.

Illustrative compounds include:

N-(hydroxymethyl)-3-(dimethylphosphono)propionamide,  
 N-(hydroxymethyl)-3-(diethylphosphono)propionamide,  
 N-(hydroxymethyl)-3-(dibutylphosphono)propionamide,  
 N-(hydroxymethyl)-3-[bis(2-chloroethyl)phosphono]  
 propionamide,  
 N-(methoxymethyl)-3-(diethylphosphono)propionamide,  
 N-(ethoxymethyl)-3-(diethylphosphono)propionamide,  
 N-(propoxymethyl)-3-(diethylphosphono)propionamide,  
 N-(isobutoxymethyl)-3-(diethylphosphono)propion-  
 amide,  
 N-(butoxymethyl)-3-(diethylphosphono)propionamide,  
 N-(hydroxymethyl)-N-methyl-3-(diethylphosphono)  
 propionamide, and  
 N-(allyloxymethyl)-3-(diethylphosphono)propionamide.

The amides of Formula I are readily produced by reaction of the corresponding N-unsubstituted amide with formaldehyde, optionally in the presence of an alcohol, in a neutral or alkaline aqueous medium at temperatures of from about 40 to about 60° C. The N-unsubstituted

amide, in turn, can be obtained by the reaction of a di-alkyl phosphite with acrylamide in the presence of a basic catalyst as described in U.S. Pat. 2,754,319.

The poly(oxymethyl)melamines which are employed in accordance with the present invention contain at least two oxymethyl groups and are represented by the formula:



wherein  $C_3N_3$  represents the s-triazine nucleus; each of  $x$ ,  $y$  and  $z$  is an integer having a value of from 0 to 3, with the proviso that the sum of  $x$ ,  $y$  and  $z$  is 3 and the compound contains at least two oxymethyl groups; and  $R^3$  is hydrogen or lower alkyl, preferably hydrogen.

Illustrative of the poly(oxymethyl)melamines are:

$N^2N^4N^6$ -tris(hydroxymethyl)melamine,  
hexakis(methoxymethyl)melamine,  
bis(hydroxymethyl)melamine,  
tetrakis(hydroxymethyl)melamine,  
pentakis(hydroxymethyl)melamine,  
bis(methoxymethyl)melamine,  
tetrakis(ethoxymethyl)melamine,  
pentakis(isobutoxymethyl)melamine, and  
tris(hydroxymethyl)tris(methoxymethyl)melamine.

In the first step of the process of this invention cellulose is treated with the  $N$ -(oxymethyl)phosphonopropionamide and an acidic catalyst to promote reaction of the phosphonopropionamide with the cellulose. Suitable acidic catalysts include hydrochloric acid, sulfuric acid and formic acid. The phosphonopropionamide and acid catalyst are preferably applied to the cellulosic substrate in aqueous solution, and when aqueous media are employed suitable catalysts include salts of strong acids and weak bases which upon hydrolysis yield acids. Ammonium halide, e.g., chloride, and various amine hydrohalides (hydrochlorides) are preferred. Other suitable catalysts are ammonium sulfate, zinc nitrate, zinc tetrafluoroborate, zinc chloride, magnesium chloride, aluminum chloride hexahydrate, ammonium oxalate and ammonium lactate. The amounts of phosphonopropionamide and catalyst present in the aqueous solution are not critical to this invention, and will depend upon the desired phosphorus content of the treated cellulose and the quantity of solution applied to the cellulose. In general, however, solutions containing from about 5 to about 35 weight percent propionamide and from about 0.5 to about 5 weight percent catalyst have been found suitable.

Insolubilization of the propionamide is effected by subjecting the thus-treated cellulose to conditions under which the propionamide reacts with the cellulose, as by heating the treated cellulose at an elevated temperature, for example, a temperature of about 150° C. to about 200° C. The heating is carried out for a period of time sufficient to effect insolubilization, usually 1 to 10 minutes. When the amide and catalyst are applied in solution, the solvent is preferably evaporated off prior to effecting insolubilization.

After insolubilization of the propionamide, the fabric is washed to remove unreacted amide, and in particular, to remove the acidic catalyst which, if left on the cellulose, would promote cross-linking of the cellulose by the poly(oxymethyl)melamine. Such cross-linking adversely affects the properties of cellulosic materials such as strength, hand and the like.

The washed fabric is then treated with the poly(oxymethyl)melamine compound and a peroxide, preferably hydrogen peroxide. This treatment, like the treatment of the first step, is preferably carried out by the use of aqueous solutions of melamine and peroxide. The concentration of melamine compound in such a solution is not narrowly critical, but should be enough to provide sufficient nitrogen to the cellulose to impart flame-retardant properties thereto, and concentrations of from

about 2 to about 25 weight percent have been found useful. Catalytic amounts of peroxide are normally in the range of from about 0.1% to about 0.5%.

Insolubilization of the melamine compound is ordinarily effected by means of wet fixation of the thus-treated material. In a preferred technique, the cellulose already modified in the first step is padded to 100%  $\pm$  30% wet pick-up with an aqueous solution containing both melamine compound and hydrogen peroxide, partially dried to a moisture content of about 10 to about 30 weight percent and then treated with steam for a period of time sufficient to insolubilize the melamine compound. Ordinarily times of from about 1 minute to about 1 hour are required.

As noted previously, the amounts of nitrogen and phosphorus necessary to give a specified degree of flame retardance are inversely related. With reference to the compounds employed in the process of this invention this relationship is defined by the expression:

20

$$N \geq 9 - 4P$$

wherein  $N$  is the weight percent nitrogen, based upon cellulose, and  $P$  is the weight percent phosphorus, based upon cellulose.

This expression applies more particularly to the use of amides which do not contain chlorine. When chlorine is present, as for example, when  $R$  is 2-chloroethyl, the nitrogen content of the fabric may be as much as 25 or 30 percent less than that specified by the foregoing expression because chlorine assists the nitrogen-phosphorus synergism with respect to flame retardance. Because the presence of halogen may adversely affect the treated cellulose its presence is not preferred.

35 In general it is preferred to employ relatively low phosphorus contents in the cellulosic product. The preference for low phosphorus concentrations is based in part upon the relatively high cost of the phosphonopropionamide as compared with melamine compound. In addition it has been found that the efficiency of the insolubilization of the phosphonopropionamide increases as the degree of add-on of the phosphonopropionamide decreases. For example, as is illustrated by Example 6, the efficiency of utilization increases from about 40% at a nominal add-on of 35 weight percent of amide to about 73% at a nominal add-on of about 16% amide. Finally, when the treatment of this invention is applied to textile products it has been found that air permeability decreases with increasing phosphorus content, and when preservation of air permeability is desired, the phosphorus content should not be in excess of about 1.8 weight percent and is desirably less than 1.2%. To provide effective flame retardance without excessive add-on of melamine compound, the cellulose should contain at least about 0.2% and preferably at least about 0.5% phosphorus.

50 When phosphorus content is within the range of 0.5 to about 1.8% the nitrogen content of the cellulose should be in the range of from 10% to about 1.7%, and preferably from about 8% to about 5%.

60 The cellulose which is treated in accordance with this invention can be from any of various sources, for instance, from seed hairs, as native cotton, from bast fabrics, as flax (linen), ramie, jute and hemp, and from regenerated cellulose, as viscose rayon. This invention also can be applied to yarns and to fabrics which are cellulosic blends, as cotton-rayon blends containing from about 10% to about 60% cotton and from about 90% to about 40% rayon. Furthermore, the invention is applicable to cellulosic yarns which then may be woven, knitted or bonded into a flame-retardant fabric with a minimum degree of impairment to characteristic properties. An additional application includes treatment of a rayon yarn or fabric which is subsequently used to manufacture a carbon yarn or fabric having improved properties and/or improved yield.

70

The following examples are illustrative. In the examples the following analytical and test methods were employed:

(1) Analyses:

(a) *Chlorine*: Saponification by means of potassium hydroxide in ethylene glycol, followed by argentometric titration of chloride ion.

(b) *Nitrogen*: Kjeldahl digestion followed by titration of distilled ammonia.

(c) *Phosphorus*: Kjeldahl digestion followed by colorimetric analysis employing acetone-water to intensify the phosphomolybdate color [Bernhart et al., *Anal. Chem.*, vol. 27, 440 (1955)].

(2) Air permeability: Federal Specifications for Textile Test Methods, CCC-T-191-b., Method 5450, reported in cubic feet per minute per square foot.

(3) Crease recovery: ASTM D 1295-60T, reported as the sum of the angles, in degrees, in warp (W) and filling (F) directions.

(4) Flame retardancy (vertical test): AATCC 34-1966, reported as char length in inches. "BEL" means burned the entire length.

(5) Flex abrasion resistance: ASTM D 1175-44T (0.5-pound head weight and 2-pound toggle tension on Stoll Flex Abrader), reported in cycles.

(6) Laundering: AATCC 88A-1964T, Test III, home-type washer, 5-pound load, full cycle, 60° C., synthetic

weight of the fabric (OWF) resulting immediately after padding are shown in the table. After padding, the samples were framed to the original dimensions, dried at 60° C., heated at 165° C. for 5 minutes to insolubilize the amide, washed, dried and conditioned as before. Weight gains were measured, and were corrected for moisture regain.

Next,  $N^2,N^4,N^6$ -tris(hydroxymethyl)melamine



10 was applied in a second step to increase the nitrogen content of the fabric by padding the samples resulting from the first step with aqueous solutions which contained both tris(hydroxymethyl)melamine (in varying amounts) and 0.3% hydrogen peroxide. Then the samples were dried to 20-30% moisture content, steamed in a laboratory steamer for 8 minutes (to hasten wet fixation), washed, dried and conditioned as before. By the procedure of wet fixation, tris(hydroxymethyl)melamine was insolubilized substantially quantitatively.

15 The results of these experiments (Samples A-G) are summarized in Table I, together with the results of an experiment in which the cotton sheeting was treated with a mixture of the amide and the melamine compound employing "Catalyst XRF" to insolubilize the reagents (Sample H). The pad-cure procedure was used in applying the mixture in a single step.

TABLE I

| Cotton sheeting sample | OWF, percent               |                            | Found in fabric sample, percent |      | Char length, inches | Stiffness (overall), mg.-cm. | Air permeability, cu. ft./min./sq. ft. |
|------------------------|----------------------------|----------------------------|---------------------------------|------|---------------------|------------------------------|----------------------------------------|
|                        | 1st step, $C_8H_{18}NO_5P$ | 2d step, $C_6H_{12}N_6O_3$ | N                               | P    |                     |                              |                                        |
| A.....                 | 29                         |                            | 5.0                             | 2.86 | 2.00                | 4.6                          | 136                                    |
| B.....                 | 29                         |                            | 7.5                             | 5.16 | 1.96                | 4.0                          | 123                                    |
| C.....                 | 20                         |                            | 5.0                             | 2.72 | 1.62                | 4.8                          | 110                                    |
| D.....                 | 20                         |                            | 9.9                             | 4.79 | 1.57                | 4.2                          | 125                                    |
| E.....                 | 20                         |                            | 12.5                            | 6.08 | 1.53                | 3.8                          | 101                                    |
| F.....                 | 11                         |                            | 13.7                            | 5.79 | 0.74                | 4.4                          | 123                                    |
| G.....                 | 11                         |                            | 16.3                            | 6.59 | 0.79                | 4.2                          | 128                                    |
| H (single step).....   | 12                         |                            | 10.6                            | 4.97 | 1.05                | 4.7                          | 366                                    |
| Control.....           |                            |                            | 0*                              | 0*   | BEL                 |                              | 97                                     |
|                        |                            |                            |                                 |      |                     |                              | 60                                     |

\*Assumed.

detergent; tumble drying. The number of laundering-drying cycles (10 or 50) is indicated by 10L or 50L, respectively.

(7) Laundering with bleach: 0.25 pint (0.5 cupful) of commercial beads based on potassium peroxymonosulfate ( $K_2SO_5$ ) was added per 16 gallons.

(8) Stiffness: (Cantilever), ASTM D 1388-64, reported in mg.-cm.

(9) Tear strength: (Elmendorf), ASTM D 1424-59, reported in pounds.

All parts and percentages are by weight unless stated otherwise.

EXAMPLE 1

Samples of all-cotton sheeting in a plain weave (bleached, desized and weighing 4.3 ounces per square yard) were conditioned at a relative humidity of 65±2% at 21±1° C. for at least 16 hours and weighed. Except for a control sample which was untreated, the samples were padded with an aqueous solution containing N-(hydroxymethyl)-3-(diethylphosphono)propionamide ( $C_8H_{18}NO_5P$ ) and, as the catalyst, an amine hydrochloride in the form of an aqueous 30% solution marketed by Millmaster Onyx Corp. under the trade name "Catalyst XRF." The concentration of "Catalyst XRF" on the weight of the bath was 3.0%. Concentrations of the reagents were varied, and the percentages on the

50 60 65 70 All of the samples treated with the amide and the melamine compounds possessed acceptable flame retardancy. Sample H, however, which was obtained by the single-step procedure, possessed a considerably increased stiffness (366 mg.-cm.) when compared with the untreated control (97 mg.-cm.) or the products of the two-step procedure of this invention (101-136 mg.-cm.). For sheeting of the type employed in this example, the stiffness should be less than about 250 mg.-cm.

The effect of increasing amounts of phosphorus on air permeability is evident from Samples A-G. Thus, at 0.74 to 0.79% phosphorus the air permeability was 52-53 ft.<sup>3</sup>/min./ft.<sup>2</sup>, whereas phosphorus contents of about 1.6% and 2% gave values of about 44 and 37, respectively. Because the permeability of the treated sheeting is desirably at least about 70% of the natural permeability, or about 42 ft.<sup>3</sup>/min./ft.<sup>2</sup>, it can be seen that phosphorus contents in excess of about 1.8 percent should be avoided.

EXAMPLE 2

Employing the general procedure of Example 1, except that the bis(2-chloroethyl) ester was used instead of the diethyl ester of N-(hydroxymethyl)-3-phosphonopropionamide, two samples were treated by the two-step method of this invention. The data for these experiments are summarized in Table II, together with the data for an untreated control.

TABLE II

| Cotton sheeting sample | OWF, percent                                                               |                                                                       | Found in fabric sample, percent |      |      | Char length, inches | Stiffness (overall), mg.-cm. | Air permeability, cu. ft./min./sq. ft. |
|------------------------|----------------------------------------------------------------------------|-----------------------------------------------------------------------|---------------------------------|------|------|---------------------|------------------------------|----------------------------------------|
|                        | 1st step, C <sub>8</sub> H <sub>18</sub> Cl <sub>2</sub> NO <sub>5</sub> P | 2d step, C <sub>8</sub> H <sub>12</sub> N <sub>4</sub> O <sub>3</sub> | Cl                              | N    | P    |                     |                              |                                        |
| A                      | 28                                                                         |                                                                       | 4.8                             | 3.15 | 2.70 | 1.46                | 5.0                          | 122                                    |
| B                      | 15                                                                         |                                                                       | 10.0                            | 1.55 | 4.36 | 0.73                | 5.6                          | 136                                    |
| Control                |                                                                            |                                                                       | 0*                              | 0*   | 0*   | BEL                 | 97                           | 60                                     |

\* Assumed.

## EXAMPLE 3

Employing the two-step procedure of Example 1, two samples (A and B) of rayon challis made of 100% viscose spun rayon in a plain weave (bleached, desized and weighing 3.8 ounces per square yard), were treated. For comparison, two additional samples (C and D) were prepared by the single-step procedure (amine hydrochloride as the only catalyst) described in Example 1. The data for these experiments are summarized in Table III, together with the data for an untreated control.

that the two-step process of this invention results in greater abrasion resistance and greater tear strength than does the single-step process. Evidence that cross-linking occurs to an appreciable extent in the single-step treatment is provided by the data for crease recovery, for crease recovery angles are significantly higher in the products obtained from the single-step process (Samples C and D) than for a corresponding add-on of chemicals in the two-step process of this invention (Samples A and B). Furthermore, the more favorable values for mechanical prop-

TABLE III

| Rayon challis sample | OWF, percent                                               |                                                                       | Found in fabric sample, percent |      |      | Char length, inches | Stiffness (overall), mg.-cm. | Air permeability, cu. ft./min./sq. ft. |
|----------------------|------------------------------------------------------------|-----------------------------------------------------------------------|---------------------------------|------|------|---------------------|------------------------------|----------------------------------------|
|                      | 1st step, C <sub>8</sub> H <sub>18</sub> NO <sub>5</sub> P | 2d step, C <sub>8</sub> H <sub>12</sub> N <sub>4</sub> O <sub>3</sub> | N                               | P    |      |                     |                              |                                        |
| A                    | 24                                                         |                                                                       | 7.5                             | 4.32 | 1.69 | 5.9                 | 80                           | 81                                     |
| B                    | 13                                                         |                                                                       | 13.3                            | 6.48 | 0.59 | 6.5                 | 124                          | 98                                     |
| C                    | 23                                                         |                                                                       | 8.0                             | 4.46 | 1.23 | 5.7                 | 290                          | 94                                     |
| D                    | 7.6                                                        |                                                                       | 16.0                            | 7.20 | 0.72 | 6.9                 | 361                          | 91                                     |
| Control              |                                                            |                                                                       | 0*                              | 0*   | BEL  | 43                  | 162                          |                                        |

\* Assumed.

## EXAMPLE 4

Employing the two-step procedure of Example 1, several samples were prepared and then laundered repeatedly with

properties which are typical of the two-step process are obtained without loss in char length or whiteness in comparison with those of the single-step process.

TABLE V

| Cotton sheeting sample | OWF, percent                                               |                                                                       | Found in fabric sample, percent | Char length, inches | Total crease recovery angles (W+F), ° | Warp Tear strength, lb. | Warp abrasion resistance, cycles | Whiteness |
|------------------------|------------------------------------------------------------|-----------------------------------------------------------------------|---------------------------------|---------------------|---------------------------------------|-------------------------|----------------------------------|-----------|
|                        | 1st step, C <sub>8</sub> H <sub>18</sub> NO <sub>5</sub> P | 2d step, C <sub>8</sub> H <sub>12</sub> N <sub>4</sub> O <sub>3</sub> |                                 |                     |                                       |                         |                                  |           |
| A                      | 20.0                                                       |                                                                       | 13.3                            | 5.28                | 1.56                                  | 4.2                     | 218                              | 179       |
| B                      | 11.0                                                       |                                                                       | 19.8                            | 7.24                | 0.78                                  | 4.5                     | 183                              | 212       |
| C                      | 20.0                                                       |                                                                       | 13.0                            | 5.89                | 1.62                                  | 4.3                     | 269                              | 244       |
| D                      | 12.0                                                       |                                                                       | 19.6                            | 7.92                | 1.36                                  | 4.2                     | 275                              | 233       |
| Control                |                                                            |                                                                       | 0*                              | 0*                  | BEL                                   | 173                     | 147                              | 3.1       |

\* Assumed.

or without persulfate bleach. To evaluate the durability of the treatment the vertical flame test was carried out before laundering and after 10 cycles. The data for these experiments are summarized in Table IV.

TABLE IV

| Cotton sheeting sample | OWF, Percent                                               |                                                                       | Found in fabric sample | Char length, inches | After 10 launderings, found in fabric sample, percent | After 10 launderings, char length, inches | After 10 launderings, char length, inches |
|------------------------|------------------------------------------------------------|-----------------------------------------------------------------------|------------------------|---------------------|-------------------------------------------------------|-------------------------------------------|-------------------------------------------|
|                        | 1st step, C <sub>8</sub> H <sub>18</sub> NO <sub>5</sub> P | 2d step, C <sub>8</sub> H <sub>12</sub> N <sub>4</sub> O <sub>3</sub> |                        |                     |                                                       |                                           |                                           |
| A                      | 10.4                                                       |                                                                       | 19.8                   | 5.77                | 5.0                                                   | None                                      | 7.30                                      |
| B                      | 10.4                                                       |                                                                       | 12.5                   | 5.28                | 4.8                                                   | K <sub>2</sub> SO <sub>4</sub>            | 5.12                                      |
| C                      | 10.4                                                       |                                                                       | 19.8                   | 3.8                 | 3.8                                                   | K <sub>2</sub> SO <sub>4</sub>            | 7.65                                      |

\* 4.8 inches after 50 launderings.

## EXAMPLE 5

The general procedure of Example 1 was followed to compare the effects on fabric properties resulting from the two-step process and from the simultaneous treatment with N-(hydroxymethyl)-3-(diethylphosphono)propionamide and tris(hydroxymethyl)melamine. The resulting samples (all made using the same type of all-cotton sheeting identified in Example 1) were subjected to several tests to evaluate the fabric treated under the different sets of conditions. By referring to Table V, below, it is evident

that samples of the same all-cotton sheeting identified at the beginning of Example 1 were padded with a variety of con-

centrations of N-(hydroxymethyl)-3-(dimethylphosphono)propionamide (C<sub>8</sub>H<sub>14</sub>NO<sub>5</sub>P) at a fairly uniform wet pick-up (106±2% WPU) so a range was obtained in the level of application on the weight of the fabric prior to curing. In each trial, the concentration of the acid-type curing catalyst, ammonium chloride, was kept constant at 4.25% on the weight of the bath (OWB). The purpose of these trials was to correlate the effect of level of application (percentage OWF) with efficiency of utilization upon insolubilization by heating for 4 minutes at approximately 170° C. The data summarized in Table VI demon-

strate that efficiency of utilization (measured here by the ratio of the percentage of phosphorus found in the fabric after curing to the percentage of phosphorus OWF before curing) is greater at lower levels of application. This economic feature is used to advantage in the present invention, which enables flame retardancy to be obtained at very low levels of phosphorus (under 1.8%) with concomitant benefits in other properties.

TABLE VI

| Cotton sheeting sample | C <sub>6</sub> H <sub>14</sub> NO <sub>3</sub> P | OWF, percent | P, percent, found in fabric sample** | Efficiency of utilization, ratio of |
|------------------------|--------------------------------------------------|--------------|--------------------------------------|-------------------------------------|
|                        |                                                  |              |                                      | (P found)/(P OWF)***                |
| A-----                 | 35.5                                             | 5.21         | 2.09                                 | 0.40                                |
| B-----                 | 25.7                                             | 3.77         | 2.07                                 | 0.55                                |
| C-----                 | 21.6                                             | 3.17         | 1.89                                 | 0.60                                |
| D-----                 | 15.6                                             | 2.29         | 1.67                                 | 0.73                                |

\*Calculated by multiplying the values in the preceding column by 0.1467, because 14.67% by weight of C<sub>6</sub>H<sub>14</sub>NO<sub>3</sub>P is phosphorus.

\*\* After curing (4 minutes at approximately 170° C.), washing to remove C<sub>6</sub>H<sub>14</sub>NO<sub>3</sub>P which did not condense with the cellulose, and drying.

\*\*\*The ratio of percentages expressed more fully is (P in the fabric after curing)/(P OWF before curing).

What is claimed is:

1. In a method for improving the flame-retardant properties of a cellulosic material by the insolubilization of an N-(oxymethyl) - 3 - phosphonopropionamide and a poly (oxymethyl)melamine on said cellulosic material, the improvement of insolubilizing said amide in the presence of an acidic catalyst and thereafter insolubilizing said melamine in the presence of hydrogen peroxide.

2. A method according to claim 1 wherein said propionamide is represented by the formula:



wherein R is lower alkyl or halogen-substituted lower alkyl; R<sup>1</sup> is hydrogen or lower alkyl; and R<sup>2</sup> is hydrogen, lower alkyl, or lower alkenyl, and said melamine is represented by the formula:



wherein C<sub>3</sub>N<sub>3</sub> represents a triazine ring; each of x, y and z is an integer having a value of from 0 to 3 with the

proviso that the sum of x, y and z is 3, and there are at least two oxymethyl groups; and R<sup>3</sup> is hydrogen or lower alkyl.

3. A method according to claim 2 wherein R is lower alkyl, each of R<sup>1</sup>, R<sup>2</sup> and R<sup>3</sup> is hydrogen, and x is 0.

4. A method according to claim 3 wherein said propionamide is employed in an amount sufficient to provide from about 0.5 to about 1.8 weight percent phosphorus, based upon cellulose, and said melamine is employed in an amount sufficient to provide from about 1.7 to about 10 percent nitrogen based upon cellulose, the nitrogen content being at least 9-4P wherein P is the weight percent phosphorus, based upon said cellulose.

5. A method according to claim 4 wherein the phosphorus content is not more than about 1.2 percent and the nitrogen content is from about 5 percent to about 8 percent.

6. A method according to claim 2 wherein said propionamide is N-(hydroxymethyl) - 3 - (dimethylphosphono) propionamide and said melamine is N<sup>2</sup>, N<sup>4</sup>, N<sup>6</sup>-tris(hydroxymethyl)melamine.

7. A method according to claim 2 wherein said propionamide is N-(hydroxymethyl) - 3 - (diethylphosphono) propionamide and said melamine is N<sup>2</sup>, N<sup>4</sup>, N<sup>6</sup>-tris(hydroxymethyl)melamine.

8. A method according to claim 2 wherein said propionamide is N-(hydroxymethyl) - 3 - [bis(2 - chloroethyl) phosphono]propionamide and said melamine is N<sup>2</sup>, N<sup>4</sup>, N<sup>6</sup>-tris(hydroxymethyl)melamine.

References Cited

UNITED STATES PATENTS

|           |         |                     |          |
|-----------|---------|---------------------|----------|
| 2,530,261 | 11/1950 | Morton et al. ----- | 8-116.2  |
| 2,781,281 | 2/1957  | Berger -----        | 117-136  |
| 3,276,897 | 10/1966 | Reeves et al. ----- | 106-15X  |
| 3,436,250 | 4/1969  | Yamaguchi et al. -- | 117-136X |

WILLIAM D. MARTIN, Primary Examiner

40 H. J. GWINNELL, Assistant Examiner

U.S. Cl. X.R.

117-136, 143, 144

UNITED STATES PATENT OFFICE  
CERTIFICATE OF CORRECTION

Patent No. 3,556,840 Dated January 19, 1971

Inventor(s) Giuliana C. Tesoro

It is certified that error appears in the above-identified patent and that said Letters Patent are hereby corrected as shown below:

Column 7, Table IV, right-hand column, "5.4" should read -- 5.1 -- and "4.1" should read -- 4.4 --. Column 9, line 1 the formula should read



Signed and sealed this 28th day of September 1971.

(SEAL)

Attest:

EDWARD M. FLETCHER, JR.  
Attesting Officer

ROBERT GOTTSCHALK  
Acting Commissioner of Pat.